

June 27, 1933.

K. J. SMITH ET AL.

1,916,026

## PROCESS FOR THE MANUFACTURE OF COKE

Filed Feb. 7, 1930



STEIN  
Inventors  
H. J. Smith  
H. V. Smith,

୧୩୫

George A. Prevost  
Attorney

## UNITED STATES PATENT OFFICE

KENNETH J. SMITH AND HOWARD V. SMITH, OF EL DORADO, KANSAS, ASSIGNEES TO  
SKELLY OIL COMPANY, OF EL DORADO, KANSAS, A CORPORATION OF DELAWARE

## PROCESS FOR THE MANUFACTURE OF COKE

Application filed February 7, 1930. Serial No. 426,619.

Our invention consists in new and useful improvements in a process for the economical manufacture of coke from fuel oil and other petroleum residuums.

5 As practical operators in the petroleum refining industry for many years, we are aware of the fact that the manufacture of coke from fuel oil and petroleum residuums is very old. We are also well acquainted with and have 10 practiced the manufacture of coke from fuel oils and petroleum residuums by means of shell stills and the commonly practiced method of producing coke in connection with oil cracking processes where the material being 15 cracked is passed through a long heated coil to a large receptacle maintained under high pressure in order to arrive at the high temperature necessary to effect cracking of the oil in the receptacle, the coke produced as a result of said operation, being a by-product.

Furthermore, we are familiar with and for some time have practiced on a large scale, the process of manufacturing synthetic coal, announced at the World's Coal Conference in 25 Pittsburgh in 1928, and described and illustrated in many technical journals shortly thereafter. In this last named process the fuel oil or petroleum residuum is heated in a long coil from whence it is partially cooled 30 and led to an open space where it is permitted to congeal into an amorphous solid comparable in many ways to bituminous coal.

The process most extensively used heretofore in the production of coke from fuel oils 35 and petroleum residuums, as before stated, has involved the use of shell stills which for obvious reasons has been found to be a costly procedure both in time and apparatus involved. In the shell still operation a still 40 is charged with several hundred barrels of fuel oil and heated externally to a very high temperature, until all of the volatile constituents are driven off and an incidental amount of cracking occurs, after which the coke is 45 removed manually from the still. In such operation the coke collecting in the bottom of the still forms an increasingly thick insulation, thereby necessitating an extremely high temperature in order to penetrate and 50 vaporize the liquid content of the still, which in a short time obviously caused burning out of the bottom of the still and necessitated repairs during which the apparatus is shut down, causing a loss of time, money and mate- 55 rial.

It is the object of our invention to overcome the disadvantages of the coking processes heretofore known, our process differing radically from any of the above in the principles applied as well as in procedure. 60

The fundamental factor of our process resides in passing the material to be treated through a pipe still and impounding sufficient heat in said material, so that, at the point of discharge from said pipe still there 65 will be a substantially complete vaporization of the volatile content without the addition of further external heat.

The main difference between our improved process and those heretofore known is that 70 we first heat the raw charging stock to the desired degree, preferably 880° F. to 925° F. but not greater than 1000° F., and then immediately transfer the same to a well-insulated coking chamber, retaining the necessary 75 heat to effect coking, without the application of additional heat to the coking chamber. The entire operation is carried on at substantially atmospheric pressure or a pressure just enough above atmospheric to force the 80 vapors and fixed gases through the vapor take-off.

In practicing our improved process we have found that the application of proper quantities of steam or other inert fluid such 85 as natural gas, oil refinery gas or flue gas, at the desired point in the pipe still, while the residuum is under heat treatment, materially assists the operation. By its presence, the steam produces a partial pressure effect or a 90 reduction of vapor pressure, thus increasing the vaporization of the residuum being treated and assisting the super-heat applied, to effect coking, thereby making it possible to operate at lower temperatures and with less 95 superheat applied to the residuum. Furthermore, the steam increases the velocity of said residuum passing through the coils.

With the above and other objects in view 100 which will appear as the description proceeds, our invention consists in the novel features herein set forth, illustrated in the accompanying drawing and more particularly pointed out in the appended claims.

The drawing illustrates diagrammatically 105 one form of apparatus which may be employed in carrying out our process, parts of said apparatus being shown in elevation and parts in section.

In the drawing, 1 represents a furnace 110

- heated by a burner 2 or any suitable means, and in which are provided a series of pipe coils 3 and 3<sup>a</sup>. 4 represents a pipe line leading from the source of fuel oil or residuum 5 and connected to the inlet end 6 of the coils 3, a suitable pump 7 being installed in said pipe line 4 for forcing the material to be treated into the coil. 8 and 9 designate well insulated coking chambers connected to the 10 discharge end 10 of the coil 3<sup>a</sup> by branch lines 8<sup>a</sup> and 9<sup>a</sup> respectively, leading from a well insulated discharge line or conduit 11 for conveying the vapors and liquids from said coil 3<sup>a</sup>.
- 15 At a suitable point anterior to the coil 3<sup>a</sup> we provide a steam inlet 12 whereby steam is injected into the heated coil during the passage of the residuum therethrough. The steam is preferably introduced into the coil at 20 a point anterior to which no coke is likely to form in the coil.

In the upper portion of the coking chambers 8 and 9 we provide vapor take-off pipes 13 leading to a condensing coil 14 which in 25 turn is directly connected to a suitable receptacle 15 in which the condensed liquids are collected, any uncondensed vapors or permanent gases entering the receptacle 15, being removed therefrom by any suitable means, 30 not shown.

In our present construction the heating coil consists of 90 tubes, of three inch inside diameter, four inch outside diameter by 24 feet long, the total coil length including 35 turn bends being about 2230 feet, with approximately 2010 feet of tubing exposed to the fire, a preheating bank 3 and a final heating bank 3<sup>a</sup>. The tubes are arranged in two banks of 45 tubes each. The charging stock 40 enters the upper or preheating bank in a counterflow direction to the ascending flue gases which have been cooled by passing around the second or lower bank 3<sup>a</sup>. The charging stock then descends to the lower 45 or final heating bank by means of the insulated connecting pipe 3<sup>b</sup> outside the furnace, and ascends in said second bank 3<sup>a</sup> from its lower extremity in a direction parallel to the travel of the flue gases. The coking chambers 50 8 and 9 are heavily insulated, horizontal, cylindrical tanks 8 feet in diameter by 25 in length.

A typical operation of our improved process was as follows:

55 Suitable charging stock such as fuel oil or petroleum residuum of 3.9° A. P. I. gravity, for example, from either crude oil stills or cracking stills was forced by the pump 7 into the heated coil 3 at the rate of approximately 60 ly 43 barrels an hour, and was preheated to a temperature preferably in excess of 400° F. during its passage through said coil. From the coil 3 the preheated oil flowed to the main heating coil 3<sup>a</sup> where it was heated to a 65 temperature ranging from 885° F. to 905° F.

Steam, at the rate of about 429 pounds per hour was continuously injected at 12 anterior to the final heating coil, into the residuum passing through the said coil 3<sup>a</sup>, the quantity of steam added varying at times, to suit conditions. 70

The mixture of steam, vapors and unvaporized material was conveyed by the relatively short-well-insulated transfer line 11 to one of the insulated receivers 8 or 9, sufficient heat being impounded in the residuum during its passage through the coil, so that, when it was discharged from said coil into the coking chamber, there was a substantially complete vaporization of the 80 volatile content. Due to the size of the chamber, the material was retained therein for a sufficient length of time to utilize the heat units impounded in the material to cause the deposition of a relatively large amount of 85 coke in said chamber. The distillate was conveyed from the coking chamber to a condenser 14 through the medium of the vapor take-off pipe 13, leaving the coke in the 90 chamber 8 or 9.

By employing a plurality of coking chambers it will be seen that we are enabled to operate a continuous process, with a continuous feed of raw material and a continuous production of coke and distillate of uniform 95 characteristics. The coke is removed from one chamber through the manhole 16, while the other chamber is in use and vice versa. The liquid products recovered in the receptacle 15 may be used for any purpose desired, as is the coke recovered from the batch still coking operation. 100

The material being treated is forced into the coils 3 and 3<sup>a</sup> at approximately 110 lbs. per square inch pressure, or a pressure below that of the injected steam at its point of injection for obvious reasons, the only function of pressure in this process being to force the charging stock through the apparatus. Our 105 process is distinguished from pressure processes in that in the former, where 110 lbs. pressure is employed as a pressure force, said pressure is merely pump pressure and is gauged at the inlet end, while in the latter 110 a pressure is maintained throughout the entire system and is gauged at the discharge end. The pressure at the discharge end of coil 3<sup>a</sup> in our process should not exceed 50 pounds per square inch for satisfactory operation. 115

In our process during a run of 12 hours, 521 barrels of residuum of 3.9° A. P. I. gravity was treated, out of which 44,739 lbs. or 120 23 per cent by weight of coke was produced, 72.4 per cent of distillate, and 4.6 per cent loss in uncondensable gases. The temperature maintained in the pipe still ranged from 885° F. to 905° F. at the outlet, and the steam injected amounted to approximately 5150 125 lbs. 130

pounds. The pressure maintained at the inlet of the coil was 125 lbs., and at the discharge end of coil 3<sup>a</sup> it did not exceed 50 pounds while the pressure in the coking chambers was about 3 lbs. gauge.

5 An analysis of the coke produced showed:

|                 | Per cent         |
|-----------------|------------------|
| Volatile matter | 13.24            |
| 10 Fixed carbon | 81.78            |
| Ash             | 4.98             |
|                 | 100.             |
| B. t. u.        | 13,853 per pound |
| 15 Sulphur      | 1.229 per cent   |

While we have described the above apparatus, operation and run in detail, they are given merely as examples, and obviously 20 other suitable apparatus for accomplishing the desired result may be employed. For example, it may be desirable to utilize the spent flue gases from the furnace to offset radiation in the coking chambers, by passing said flue 25 gases underneath and around said chambers on their way to the stack. These flue gases are purely an additional insulating medium for further guarding against the dissipation of the heat impounded in the material dis- 30 charged into the coking chambers and are not to be considered as additional external heat, the heat from said gases being insufficient to in any way effect the reaction in the chambers.

35 It will be noted that in actual practice the raw charge may be preheated by means of a heat exchanger which transfers the heat from the hot vapors leaving the coking chambers, to the raw charge before it enters 40 the coil 3<sup>a</sup>, thus eliminating the preheating coil 3.

In practicing our process, the temperatures, pressures and proportions may also be varied to suit conditions, the temperature of 45 the pipe still being controlled and varied according to the character of the raw charge to be treated.

From the foregoing it will be seen that 50 our improved process possesses all of the advantages of the standard coking still operation with very few, if any, of its disadvantages. As may be readily seen, an installation of apparatus suitable for conducting our process can be made in which the investment 55 is small, the capacity high with the maximum furnace efficiency, the maintenance cost far below the ordinary and the cleaning costs much less than the standard coking still operation.

60 The result obtained by our process, and not obtained in any of those with which we are familiar is that through the use of super-heat, aided by the injection of steam, we are able to reduce the volatile matter remaining 65 in the coke to a minimum thus producing a

high quality coke, directly comparable with other petroleum cokes and for which there are established markets.

Furthermore, our process affords almost 70 unlimiting flexibility in charging stock and the character of the product produced, as by varying the coil outlet temperature we are able to obtain coke of any desired volatile content. It will also be noted that we have experienced no difficulty due to coke forming 75 in the coil.

By such terms as "heavy residuum hydrocarbon oil" and "petroleum residuum", in the 80 claims, we mean such charging stock as fuel oil or petroleum residuum from either crude oil stills or cracking stills.

From the above it is believed that our process may be readily understood by those skilled in the art without further description, it being borne in mind that numerous 85 changes may be made in the details of construction and operation without departing from the spirit of the invention as set forth in the following claims.

What we claim and desire to secure by Letters Patent is:

1. The process of treating heavy residuum hydrocarbon oil for the production of an optimum yield of coke, which comprises pre-heating said oil and forcing the same 95 through an elongated passageway of restricted cross sectional area, heating said oil during its flow through said passageway, injecting a suitable heated gaseous fluid which is chemically inert, into said oil at a point anterior to the last named heating step, transferring the resulting mixture without any substantial loss of heat, from said passageway to an expansion zone, and maintaining the mixture in said zone for a sufficient 100 length of time to utilize the heat units impounded therein, to cause the deposition of an optimum amount of coke from said mixture, said oil being heated in said passageway to temperatures insufficient to materially crack the oil during its flow through said 105 passageway, but sufficient to cause a substantially complete vaporization of the volatile content of said oil at the outlet of said passageway, the pressure on said mixture at the 110 outlet of said passageway not exceeding 50 pounds per square inch.

2. The process of treating heavy residuum hydrocarbon oil for the production of an optimum yield of coke, which comprises pre-heating said oil and forcing the same 120 through an elongated passageway of restricted cross sectional area, heating said oil during its flow through said passageway, to temperatures from 880° F. to 925° F., injecting a suitable heated gaseous fluid which is chemically inert at said temperatures, into said oil at a point anterior to said last named heating step, transferring the resulting mixture without any material cracking having 125 130

taken place and without any substantial loss of heat but substantially in vapor form, from said passageway to an expansion zone, and maintaining the mixture in said zone for a sufficient length of time to utilize the heat units impounded therein, to cause the deposition of an optimum amount of coke from said mixture, the pressure on said mixture at the outlet of said passageway not exceeding 50 pounds per square inch and the pressure in said expansion zone being only slightly in excess of atmospheric pressure.

3. The process of treating a heavy petroleum residuum from a cracking still or the like for the production of an optimum yield of coke, which comprises preheating said residuum and forcing the same through an elongated passageway of restricted cross sectional area, heating said residuum during its flow through said passageway, to temperatures from 880° F. to 925° F., maintaining a pressure at the outlet of said passageway not exceeding 50 pounds per square inch, injecting a suitable heated gaseous fluid which is chemically inert at said temperatures, into said residuum at a point anterior to said last named heating step, transferring the resulting mixture without any material cracking having taken place and without any substantial loss of heat, from said passageway to an expansion zone, wherein a substantially complete vaporization of the volatile content of the mixture occurs, without the addition of further external heat, and maintaining the mixture in said zone for a sufficient length of time to utilize the heat units impounded therein, to cause the deposition of an optimum amount of coke from said mixture, the pressure in said expansion zone not greatly exceeding atmospheric pressure.

4. The process of treating a heavy petroleum residuum from a cracking still or the like for the production of an optimum yield of coke, which comprises preheating said residuum and forcing the same through an elongated passageway of restricted cross sectional area, heating said residuum during its flow through said passageway, to temperatures from 880° F. to 925° F., maintaining a pressure at the outlet of said passageway not exceeding 50 pounds per square inch, injecting a suitable heated gaseous fluid which is chemically inert at said temperatures, into said residuum at a point anterior to said last named heating step, transferring the resulting mixture without any material cracking having taken place and without any substantial loss of heat, from said passageway to an expansion zone, wherein a substantially complete vaporization of the volatile content of the mixture occurs, without the addition of further external heat, maintaining the mixture in said zone for a sufficient length of time to utilize

the heat units impounded therein, to cause the deposition of an optimum amount of coke from said mixture, the pressure in said expansion zone not greatly exceeding atmospheric pressure, and withdrawing and condensing the vapors from said zone.

5. The process of treating heavy residuum hydrocarbon oil from a cracking still or the like for the production of an optimum yield of coke, which comprises preheating such residuum and forcing the same through an elongated passageway of restricted cross sectional area, heating said residuum during its flow through said passageway to temperatures from 880° F. to 925° F., injecting steam into said residuum as the latter travels through said passageway, immediately transferring the resulting mixture without any substantial loss of heat, from said passageway to an expansion zone, wherein a substantially complete vaporization of the volatile content of the mixture occurs, without the addition of further external heat, and maintaining the mixture in said zone for a sufficient length of time to utilize the heat units impounded therein, to cause the deposition of a relatively large amount of coke from said mixture, the pressure at the outlet of said passageway being super-atmospheric but not exceeding 50 pounds per square inch and the pressure in said expansion zone not materially exceeding atmospheric pressure.

6. The process of treating heavy residuum oil for the production of an optimum yield of coke, which comprises forcing such oil through an elongated passageway of restricted cross sectional area, heating said oil during its flow through said passageway, to temperatures from 880° F. to 925° F., injecting a suitable gaseous fluid which is chemically inert at said temperatures, into said oil at an intermediate point in said passageway after said oil has been preheated in said passageway, transferring the resulting mixture without any material cracking having taken place and without any substantial loss of heat, from said passageway to an expansion zone, where a substantially complete vaporization of the volatile content of the mixture occurs, without the addition of further external heat, maintaining the mixture in said zone for a sufficient length of time to utilize the heat units impounded therein, to cause the deposition of an optimum amount of coke from said mixture, and withdrawing and condensing the vapors from said zone, the pressure at the outlet of said passageway not exceeding 50 pounds per square inch and the pressure in said expansion zone not materially exceeding atmospheric pressure.

In testimony whereof we affix our signatures.

KENNETH J. SMITH.  
HOWARD V. SMITH.